

May 13, 1930.

H. J. CORDY ET AL.

1,758,188

#### METHOD OF ROASTING FINES

Filed Jan. 30, 1928.



## UNITED STATES PATENT OFFICE

HENRY J. CORDY AND WILLIAM J. BURGOYNE, OF SULPHIDE, ONTARIO, CANADA,  
ASSIGNORS TO GENERAL CHEMICAL COMPANY, OF NEW YORK, N. Y., A CORPORATION OF NEW YORK

## METHOD OF ROASTING FINES

Application filed January 30, 1928. Serial No. 250,616.

Our invention relates to the roasting of finely divided sulphide ores, flotation concentrates and the like, and more particularly to a method of roasting finely divided pyrites 5 ores or flotation concentrates, to thoroughly desulfurize the same and to produce sulfur dioxide for use in the manufacture of sulfuric acid.

The present practice in pyrites fines roasting generally involves the use of mechanically operated multiple hearth constructions, such, for example, as the well known MacDougal, Herreshoff, and Wedge burners, and while these burners provide a very 10 effective roasting of the fines, their complicated construction and operation involves considerable initial and maintenance expense.

As distinguished from the "bed" roasting operation of these burners, it has been suggested to roast the fines while in gaseous suspension, wherein the fines are either injected 15 into a roasting chamber in suspension in the oxidizing gas, or are simply showered downwardly into the roasting chamber wherein 20 they encounter cross or counter currents of the suspending gas.

This suspension roasting is best applicable when the fines are in a very finely divided state, e. g. as flotation concentrates, and it 25 presents the notable advantage over the mechanical multiple hearth operation of considerably lowering the cost of production, by reason of the elimination of the involved and expensive rabbling and other apparatus which 30 distinguishes the construction and operation 35 of the mechanical burners. In the practice of this suspension roasting, however, and particularly as applied to roasting pyritic fines, difficulties of some moment are presented 40 which must be overcome before the obvious theoretical advantages of this type of operation are practically available.

The most serious and perplexing difficulty 45 encountered in the suspension roasting of pyrites fines is the objectionable formation of accretions or "scar" on the walls of the roasting chamber during the roasting operation. These scar masses assume imposing proportions with disconcerting rapidity, and in a 50 relatively short time masses weighing several

hundred pounds are commonly formed. Unless these masses are removed, obstruction of the roasting passage will result and the operation will be otherwise seriously hindered. The scar masses may be manually broken 55 away, or "barred" down, from the walls periodically, but the frequency with which this operation must be repeated to keep the scar formation within reasonable limits results in inordinate interruption of the operation, 60 and, in addition, the wear and tear on the apparatus occasioned by the heavily falling masses raises even more serious objection to this manner of removal. Moreover, the problem of incomplete desulphurization is 65 not solved thereby, for the considerable amounts of undesulphurized material which are confined within the accretions pass off in the cinder substantially unaffected.

We have investigated the scarring problem noted and, while the exact reason for its occurrence is rather difficult to determine, it would seem to be more or less ascribable to the very pronounced tendency which the iron pyrites exhibits to sinter at a particular stage 70 of its desulphurization, at which stage it readily adheres to the confines of the roasting chamber and builds up accretions thereon. Investigation of a typical iron-pyrites ore in this relation appeared to indicate that a point 75 in its transition from  $FeS_2$  to  $Fe_2O_3$ , which would roughly correspond to the oxidation of one atom of the sulphur in the  $FeS_2$ , the partially desulphurized material sinters much more readily than at prior or subsequent 80 stages in the desulphurization. This may be explained either on the basis that  $FeS$  is the major form existing at this particular stage and that the  $FeS$  per se sinters much more readily than any of the other transition or 85 final products, or possibly that there is a formation of a eutectic of  $FeS$  and  $Fe_2O_3$ .

Regardless of the exact reasons for this behavior, however, the results of our determinations have clearly indicated that the 90 solution of this problem rests in so controlling the operation that the pyrites being roasted will not be permitted to contact with the walls of the reaction chamber while it is 95 in the transitory sticky condition noted.

We have experimented with various methods of roasting the pyrites fines in suspension, in an endeavor to find a means of overcoming the effect of this transitory sintering condition, and we have found that by injecting a quantity of the oxidizing gas adjacent the walls of the roasting chamber in the upper part thereof, that scarring of the chamber walls is eliminated, very thorough desulphurization of the fines is obtained, and concentrations of sulfur dioxide are obtainable which are very suitable for use in the manufacture of sulphuric acid. This action appears to be due to the interposition of a supplemental portion or blanket of the oxidizing gas between the walls of the roasting chamber and the main suspension of the burning pyrites when the latter is in the state conducive to scar formation.

In the following specification we have described in detail a specific manner in which the invention may be applied, and one embodiment of the apparatus utilizable therein is shown in the accompanying drawing in which:

Figure 1 is a sectional elevation of a pyrites burner for carrying out our invention.

Figure 2 is a plan view of a portion of the feeding mechanism for the same taken along the line 2—2, Figure 1, and

Figure 3 is a plan view of another portion of the feeding mechanism taken along the line 3—3, Figure 1.

Referring to the drawing, and in particular to Figure 1, reference numeral 4 indicates a shaft burner comprising a shell 5, constructed of a suitable refractory material such as fire brick or the like, which defines a roasting chamber 6 of cylindrical shape throughout the major portion of its length. A casing 7 of steel or similar material is provided about the sides of the shell 5 to suitably reinforce the same. Chamber 6 is provided, with a feed inlet 8 in the center of the burner crown 9; a trough-like cinder pit 11, constituting the bottom of the chamber, which extends diametrically thereacross and is open at the base throughout its length to provide an elongated cinder outlet 12; and a lateral gas outlet 13 in the wall of the chamber just above the cinder pit 11. Suitably constructed work holes 14, 15 and 16 covered by detachable external closures 17, 18 and 19 are also provided to afford access to the interior of the roasting chamber.

Terminating in the feed inlet 8 is a feed mechanism 20 for introducing the fines and oxidizing gas into the roasting chamber. This feed mechanism is constructed as follows: A charging hopper 21, into which the finely divided material to be roasted is introduced in any suitable manner, is mounted above and terminates in a tubular charging conduit 22, which conduit discharges into a

cross 23. This cross comprises a lateral arm 24 to which is bolted a cap 25 provided with a suitable bore for the accommodation of conduit 22; a downwardly extending arm 26 above which the discharging end of the conduit 22 terminates; a lateral arm 27 to which is bolted a cap 28 having a bearing 29; and an upwardly extending arm 31 having a cap 32 detachably attached thereto in any well-known manner whereby access may be readily had to the interior of the cross. Within the conduit 22 is a helicoid conveyor 33 whose shaft 34 is mounted for rotation in bearing 29 in cap 28 and bearing 35 provided in a plate 36 closing one end of the conduit 22.

A cylindrical coupling 37 having top and bottom flanges 38 and 39 respectively, is secured at its top flange 38 to the flanged bottom 41 of the arm 26 of cross 23, and retained intermediate the joined flanges 38 and 41 is a baffle plate 42 which extends completely across the passage provided by coupling 37. Baffle plate 42 is provided with a central orifice 43, and below and in alignment with said orifice is a distributing cone 44 supported by a cross beam 45 which extends diametrically across and is bolted or otherwise secured to the coupling 37 in any well-known manner. A rod 46 depends from the cone 44, extending through a bore provided therefor in the cross beam 45, and this rod terminates at its lower end in a larger distributing cone 47.

Another cylindrical coupling 48 having top and bottom flanges 49 and 50 respectively, is bolted to coupling 37 through the medium of the flanges 49 and 39, and gripped intermediate the joined flanges is the flanged top 51 of a funnel 52.

A cylindrical casing 53 having top and bottom flanges 54 and 55 respectively, is bolted to coupling 48 through the medium of the flanges 54 and 50, and has its bottom flange 55 mounted upon and bolted to the top flange 56 of a cylindrical sleeve 57 which is set snugly into the feed inlet 8 and is supported therein by means of a circumferential projection 58 which abuts against the surface of the crown 9.

A terminal cylinder 59 is suspended by means of its top flange 59' gripped between the joined flanges 54 and 50, and terminates at a point below the base of the distributing cone 47, said cylinder forming a substantial continuation of the vertical passage provided by the super-jacent couplings 48, 37 and the arm 26 of cross 23.

A cylindrical gas-distributing sleeve 60, having a top flange 61 is carried on the headed ends 62 of a number of suspension rods 63 extending through said flange, at least four of said rods spaced equi-distantly around the flange 61 being ordinarily desirable. These rods extend through suitable bores provided in flanges 54 and 50 and are re-

tained on the latter by means of adjustable nuts 64 on their threaded ends 65, whereby the sleeve 60 may be adjusted vertically of the cylinder 59 and the inlet sleeve 57. The sleeve 60 extends around the lower portion of the cylinder 59 in uniform radially spaced relation thereto whereby a narrow annular gas passage 66 is provided between the cylinder and the sleeve, and the clearance thereby presented will permit the sleeve to be readily adjusted vertically of the cylinder. The sleeve 60 is also positioned in uniform radially spaced relation to a portion of the casing 53 and the inlet sleeve 57, which members surround sleeve 60, and an additional annular gas passage 67 is thereby provided between the sleeve 60 and these surrounding members. The annular mouth 68 of this latter passage 67 is defined by the rim of the flanged bottom 69 of sleeve 60 and the adjoining inner surface of the inlet sleeve 57, and by suitable vertical adjustment of the sleeve 60 by means of the suspension rods 63 the size of the mouth 68 may be varied as desired, whereby a greater or less amount of oxidizing gas may be admitted therethrough into the roasting chamber from the passage 67.

As shown in Figs. 1 and 3, a series of suitably spaced apertures 71 for entrance of the oxidizing gas is punched inwardly in the wall of the sleeve 60 at points therein below the bottom of cylinder 59, all of which apertures give access to the interior of the sleeve in substantially the same general direction as regards the circumference of the sleeve. Spaced lower down in the wall of the sleeve is another series of similar inwardly punched apertures 72 which give access to the interior of the sleeve in a direction substantially opposite to that of the upper series. A tangential extension 73 (Fig. 2) projects from the casing 53, and to the flanged end 74 of said extension is bolted the flanged end 75 of a pipe 76 leading from a suitable fan blower (not shown), whereby the oxidizing gas may be blown into the feed mechanism.

Beneath the cinder outlet 12 and extending in diametrical alignment therewith is a discharge conduit 77 in which is mounted in any suitable fashion a helicoid conveyor 78 for continuously removing the cinder from the burner. A grate 79 is mounted above the cinder outlet 12 leading into the discharge conduit, which grate may be supported at its sides by lugs 80 on the inclined walls 81 of the trough-like cinder pit 11, or in any other suitable fashion. By means of the grate 79 pieces of cinder too large to be conveniently handled by the conveyor may be periodically broken up by a workman to permit their passage through the grate. Access to the grate for the operation noted is afforded by the work hole 14.

The gas outlet 13 leads to a dust chamber 82 of any well-known type, part of which is

shown in Figure 1, wherein the gases are separated from the entrained dust prior to their utilization in the manufacture of sulphuric acid. In view of the fact that it is desirable to maintain a substantially neutral, (i. e., atmospheric) or a slightly positive pressure above the cinder outlet 12 as noted in detail hereinafter, provision must be made for drawing the dust-laden gases through the dust chambers, and this may be accomplished by maintaining a suitably reduced pressure at the outlet for the dust-free gases from the dust chambers (not shown), by any well-known means such as a fan blower.

The operation of our invention is substantially as follows: The furnace is first strongly preheated, for example by means of one or more oil burners inserted through the work hole 14, until a temperature is obtained in the chamber 6 substantially above the ignition point of the iron pyrites, for example, about 850° C. During the preheating operation work holes 15 and 16 are uncovered to provide flues for the escape of the products of combustion.

Finely divided iron pyrites, which has been dried until the moisture is not greater than 0.3% and preferably between 1% and 2%, and of a particle size such that 100% will pass a 60 mesh (to the inch) screen, is then fed into the hopper 21, in any suitable manner. From the hopper the fines are substantially continuously supplied to the helicoid conveyor 33 within the charge conduit 22, by means of which they are delivered into the passage in the arm 26 of cross 23. Some of the pyrites fines will pass directly through the orifice 43 in the baffle plate 42, and the remainder will pile up around the orifice until a funnel-like mass of fines is formed with the orifice 43 as its mouth, which mass will aid in directing subsequent portions of fines to the orifice and onto the distributing cone 44. Passing over the cone 44, the fines will be directed onto the sides of the funnel 52, and thence will proceed into the terminal cylinder 59, at the lower portion of which they will be spread out by the distributing cone 47 into a somewhat cylindrical-shaped sheet, in which form they will reach the gas distributing sleeve 60.

Air or oxygen may be used as the oxidizing gas, preferably the former, and either at atmospheric temperature, or preheated to any desired degree thereabove which is below the ignition point of the pyrites, is blown through the pipe 76 and tangentially into the space between the casing 53 and the cylinder 59 (Figures 1 and 2). The amount of air introduced will depend upon the amount of sulfur in the fines to be desulphurized, the concentration of SO<sub>2</sub> desired in the exit gases, and other factors evident to one skilled in the art, and the regulation of the air supply may be accomplished in any suitable and well-known manner. In practice, determi-

nation of the  $\text{SO}_2$  content of the exit gases and the character of the cinder will usually indicate the necessary regulation of the air supply to provide the desired results, the fines being supplied at a substantially regular rate. The pressure under which the air is introduced should be so regulated that a positive pressure very closely approaching atmospheric is obtained over the cinder outlet, a slight plus pressure of about .02" to .03" being suitable under most circumstances.

Upon introduction into the feed mechanism the air will whirl around the cylinder 59, and traveling downwardly, a major portion of the same will pass into the interior of the air distributing sleeve 60 through the passage 66 and the apertures 71 and 72 leading off passage 67, and the remainder will sweep directly into the roasting chamber 6 through the mouth 68 of passage 67. The distributing sleeve 60 should be so adjusted by means of its suspension rods 63 that the size of the mouth 68 is such that only sufficient air is admitted therethrough to prevent scar formation on the walls of the roasting chamber. This can be determined by varying the size of the mouth and observing the effect upon the chamber walls through one of the work holes 15 or 16. The amount of scar inhibiting air necessary is usually a minor proportion of the total amount of air admitted. The sheet of pyrites fines showering out of the terminal cylinder 59 will be swept up in the turbulent air pouring into the sleeve 60 and the substantial suspension of the intimately mixed air and fines obtained thereby, will pass on into the hot roasting chamber 6. Upon entering the preheated chamber the suspension of fines and air will be ignited and oxidation will thereafter proceed at a very rapid rate.

The oxidation of the iron pyrites is a strongly exothermic reaction, to the extent that it is substantially self-sustaining, and other than the necessity of initiating the reaction, for example, by preheating the furnace to a suitable temperature above the ignition point of the pyrites, no auxiliary heat is required. In operation the temperature will be quite high throughout the chamber 6; in the production of an approximately 10%  $\text{SO}_2$  gas, from a typical iron pyrites ore, for example, the temperature in the roasting chamber was in the neighborhood of  $1000^\circ \text{C}$ .

Upon the entry of the turbulent gaseous suspension into the enlarged space presented by the roasting chamber, expansion of the suspension takes place, and this expansion is enhanced by the large amount of heat supplied by the combustion of the fines in addition to that emanating from the heated walls of the roasting chamber. This expansion tends to cause an appreciable proportion of the suspended particles to be thrown toward the chamber walls, and such particles as are

in the transitory sticky condition hereinbefore discussed would under ordinary circumstances tend to adhere to the walls upon contacting therewith and rapidly build up accretions thereon.

The portion of air, however, which enters the roasting chamber through the annular mouth 68, simultaneously with the introduction of the main body of the suspension from the sleeve 60 serves to inhibit throughout the operation the usually inescapable scar formation.

The initial stages of the roasting operation are the most intense and normally take place in the upper part of the roasting chamber. It is in this upper part of the chamber that the tendency toward scar formation appears to be most marked, and it seems probable that as the proportion of the  $\text{Fe}_2\text{O}_3$  increases, the tendency toward scarring decreases. On that basis it would seem that the provision of the air blanket between the walls of the chamber and the burning suspension need only be confined to the upper part of the chamber in order to prevent scar formation, and it may be that such is the case in the operation of the present method as noted, although the particular path of the air blanket is more difficult to trace the greater its penetration into the furnace. On the other hand it is quite possible that the gaseous suspension of fines could be introduced under such pressure, for example, that the scar forming stage would occur at a point considerably lower down in the roasting chamber, in which event it would be necessary to run the air blanket substantially throughout the length of the chamber.

In view of these considerations it is essential primarily that the air blanket be interposed between the walls of the chamber and the burning pyrites while the latter is in a state conducive to scar formation, regardless of its relative location in the roasting chamber while in that state. That such is the case in the operation of our method is evidenced by the fact that by suitably varying vertically the position of the flanged sleeve 60, and thereby the volume and direction of the air blanket admitted through the mouth 68, the formation of scar under such variations of the roasting operation as are involved in ordinary industrial practice can be eliminated.

Whether the scar inhibiting action of the air blanket is due to an oxidizing effect, whereby the particles in the sticky stage are oxidized past that stage prior to contacting with the chamber walls, or to a physical effect involving entrainment of the particles, whereby they are prevented from contacting with the walls, or to a combination of both effects, is practically indeterminate and not particularly material. Regardless of the exact explanation it is certain that this auxil-

iary portion of the oxidizing gas is interposed in the upper portion of the furnace between the walls of the chamber and the burning fines while they are in a state conducive to the formation of scar on the walls.

5 The length of the roasting chamber and the speed of introduction and travel of the fines and air should be such that a thorough desulphurization is obtained in the passage 10 through the roasting chamber, as is obvious to one skilled in the art.

By conducting the operation in accordance with the foregoing principles, the fines in suspension are quite thoroughly desulphurized by the time the cinder and gas outlets 15 are reached, and by regulation of the pressure as hereinbefore noted, the major portion of the desulfurized particles, mainly in the form of iron oxide collects in the cinder pit 20 whence it is conducted away by the helicoid conveyor 78. The gases containing the SO<sub>2</sub> passing into the dust chambers 82 carry entrained therein an appreciable portion of the finest particles, i. e. dust, consisting mainly of iron oxide is collected in 25 the dust chambers, and the dust-free gases containing the SO<sub>2</sub> are drawn from the chamber and conducted away for utilization in the production of sulphuric acid.

30 The roasting of pyritic fines in suspension according to our invention provides an operation which, in practice, presents numerous advantages over the various methods of burning such fines heretofore suggested.

35 Its most important accomplishment is the removal of the obstacle to efficient practical operation presented by the formation of the objectionable scar. The sulfide fines are, moreover, very thoroughly desulphurized, a 40 very desirable feature from an efficiency standpoint; this very thorough desulphurization being also ascribable in the main to the elimination of the scar formation which serves to prevent thorough desulphurization 45 of the pyrites fines.

In addition, the operation requires but a slight amount of attention, and the initial and maintenance expense involved are such as to permit production at a very low cost.

50 While we have specifically noted the application of our invention to the roasting of finely divided iron pyrites ore or flotation concentrate, it is obvious that our invention is not confined to the use of that particular 55 material but is applicable generally to other sulphide ores where the undesirable formation of similar scar is involved. Copper pyrites ore and flotation concentrates of the same are characterized by a similar action, 60 and the same is also true of pyrrhotite although to a less marked degree.

We claim as our invention:

1. The method of roasting a finely divided sulphide ore which comprises forming a suspension of said ore in an oxidizing gas, and

burning said suspended ore in a roasting chamber while maintaining a portion of said gas between the walls of said chamber and said burning ore while the latter is in a state conducive to scar formation on said walls, 70 whereby said scar formation is avoided.

2. The method of roasting a finely divided sulfide ore which comprises forming a suspension of said ore in an oxidizing gas, introducing said suspension into a roasting 75 chamber at a temperature sufficient to ignite said suspended ore and to permit substantial completion of the desulfurization thereof, and maintaining a supplemental portion of said gas between the walls of said chamber 80 and said burning ore while the latter is in a state conducive to scar formation on said walls.

3. The method of roasting a finely divided sulfide ore which comprises dividing a body 85 of oxidizing gas into two portions, suspending said finely divided ore in one of said portions, introducing said suspension into a roasting chamber at a temperature sufficient to cause ignition of said ore, and introducing 90 the other portion of said oxidizing gas into said chamber between the walls thereof and the burning ore in suspension when in a state conducive to scar formation on said walls.

4. The method of roasting a finely divided sulfide ore which comprises forming a suspension of said ore in an oxidizing gas, burning said suspended ore in a chamber, and maintaining a portion of said gas between the walls of said chamber and said burning ore 100 to a point in said chamber where sufficient oxidation of said ore has taken place to inhibit the subsequent formation of scar on said walls.

5. The method of roasting a finely divided sulfide ore which comprises contacting said finely divided ore with a turbulent portion of a body of air whereby said ore is substantially suspended in said portion, passing said suspended ore into a roasting chamber, igniting said suspended ore therein, and simultaneously with the resultant combustion of said ore passing another portion of said body of air between the walls of said chamber and that portion of the burning ore which is in 110 a state conducive to the formation of scar on said walls.

6. The method of roasting a finely divided sulfide ore which comprises forming a suspension of said ore in air, passing said ore into 120 a roasting chamber at a temperature at which self sustaining combustion of the same will be initiated and maintained, maintaining a blanket of air between the walls of said chamber and said burning ore while in a state conducive to scar formation on said walls, retaining said suspension in said roasting chamber a sufficient period to result in substantial desulphurization of the sulfide ore, and separating the desulfurized ore from the gases. 125 130

7. The method of roasting a finely divided sulfide ore which comprises bringing said ore in contact with a turbulent body of air at a temperature below the ignition point of said ore to form a substantial suspension of the ore in the air, passing said suspension into a roasting chamber at a temperature above the ignition point of said ore whereby combustion of said suspended ore will be initiated, and simultaneously passing a blanket of air completely around and in contact with said suspension and between said burning suspension and the walls of said chamber, said air blanket being in sufficient quantity and of such extent of intervening contact with said suspension and said walls to inhibit the formation of scar on said walls by portions of said burning ore throughout the passage of said ore through said chamber. 70
8. The method of roasting a finely divided sulfide ore which comprises forming a suspension of said ore in an oxidizing gas, introducing said suspension into a roasting chamber at a temperature sufficient to ignite said suspended ore, and enveloping said suspension at the point of introduction into said chamber in a supplemental portion of said oxidizing gas, whereby scar formation on the walls of said chamber is avoided. 75
9. The method of roasting a finely divided sulfide ore which comprises forming a suspension of said ore in an oxidizing gas, introducing said suspension into the upper part of a roasting chamber at a temperature above the ignition point of said suspended ore, enveloping said suspension at the point of introduction of said suspension into said chamber in a downwardly moving supplemental portion of said oxidizing gas, and passing said burning ore downwardly through said chamber until substantial desulphurization of said ore is obtained. 80
10. The method of roasting a finely divided sulfide ore which comprises forming a suspension of said ore in an oxidizing gas, introducing said suspension into a roasting chamber at the upper part thereof, simultaneously introducing a supplemental portion of said oxidizing gas adjacent the walls of said chamber at the upper part thereof, igniting said suspended ore substantially upon its introduction, and passing said burning ore downwardly through said chamber until the desired degree of desulphurization is obtained. 85
11. The method of roasting a finely divided sulfide ore which comprises forming a suspension of said ore in an oxidizing gas, and burning said suspended ore in a roasting chamber while maintaining a layer of gas between the walls of said chamber and said burning ore while the latter is in a state conducive to scar formation on said walls, whereby said scar formation is avoided. 90
12. The method of roasting a finely divided sulfide ore which comprises forming a suspension of said ore in an oxidizing gas, introducing said suspension into a roasting chamber at a temperature sufficient to ignite said suspended ore, and enveloping said suspension at the point of introduction into said chamber in a supplemental portion of gas, whereby scar formation on the walls of said chamber is avoided. 95
- In testimony whereof, we affix our signatures. 100
- HENRY J. CORDY. 105
- WILLIAM J. BURGOYNE. 110